

## UNITED STATES PATENT OFFICE

2,583,269

PROCESS FOR DYEING ONLY THE FLESH  
SIDE OF CHROME-TANNED FUR SKINS

Ernst Lüscher and Albert Engeloch, Basel, Switzerland, assignors to Sandoz A. G., Basel, Switzerland, a Swiss firm

No Drawing. Application August 26, 1949, Serial  
No. 112,646. In Switzerland August 30, 1948

3 Claims. (Cl. 8—10)

**1**  
The present invention relates to a method of dyeing fur skins with reserve of the wool- or hair-fur, which method consists in that lamb, sheep, or other hair skins which have been preferably or exclusively tanned with chromium compounds and the flesh side of which is gently buffed are dyed, preferably at a temperature of 40–50° C., in an aqueous solution in the presence of capillarily active organic compounds with preferably substantive dyestuffs dyeing only the flesh side.

Fur skins are obtained by this process the flesh side of which is dyed while the wool- or hair-fur remains undyed. If this latter has also to be dyed it can be done by using suitable dyestuffs in the same or in a fresh bath.

If an equal or two colour effect is desired wherein leather and wool- or hair-fur are to be dyed equally or differently respectively it is preferably done by addition of acetate silk dyestuffs to the dyebath.

As capillarily active organic compounds there may be used: soaps and synthetic capillarily active organic substances, for example alkylbenzene and alkylnaphthalene sulfonic acids, fatty alcohol sulfonates and fatty acid condensation products such as oleic methyltauride, the oleic esters of hydroxyethanesulfonic acid and the sulfonates of glycerol-monooleate esters. These products are added to the baths in amounts of 0.25–3 grams per liter of dyebath.

The pretreatment of the leather preceding the dyeing operation, namely the milling of the undyed fur- or hair-skins, is conveniently done in a bath which also contains capillarily active compounds, such as for instance those mentioned above. The subsequent dyeing of the leather can be effected in a fresh bath or in the pretreating bath itself.

As dyestuffs preferably those substantive dyestuffs are used which themselves exert a good preserving action on the wool- and hair-fibres and which dye the leather well.

If a more penetrating dyeing is desired it can be obtained by adding ammonia to the dyebath until the pH-value amounts to 9.2 at most and by acidifying the dyebath shortly before dyeing is completed until a pH value of 3.3 at least is reached.

In case where greater lots are to be dyed the dyebath can further be used after the consumed amounts of dyestuffs and the capillarily active substances have been supplied. If a dyebath which, in view of a more penetrating dyeing, is first rendered alkaline and then acid, is desired for another bath it must also be adjusted by means of ammonia to a pH value of 9.2 at most.

**2**  
The present dyeing method is particularly suitable for chromium tanned lamb- and sheep-skins. Skins tanned in combination with synthetic or vegetable tanning agents are less suited as, owing to poor affinity for the dyestuffs, no full shades are obtained.

In case the wool shows a light dyeing it is preferable to manually wash the skins in a bath containing 5 grams of a fatty alcohol sulfonate per 10 each liter of bath, to rinse the same, and to subsequently centrifuge and dry them.

The following examples without being limitative in any way show how the above process may be carried out in practice.

**15**  
*Example 1*  
75 pieces of sheep skins of a medium size gently buffed on the fleshside and tanned in the conventional way exclusively or preferably with 20 chromium compounds were placed in a paddle of 1000 litres of water at a temperature of 35° C. containing 0.5–1 gram/litre of lauryl alcohol sulfonate, agitated for a short time and then allowed to remain in the dyebath over night. On the 23 next day the skins were pulled through squeezing rolls or centrifuged. The thus pretreated skins were now put in a paddle containing 1000 litres of water at 48° C. and 1.5–2 grams/litre of lauryl alcohol sulfonate where they were agitated for 30 about 5 minutes. Now an aqueous solution of 1 kilogram of "Solar Brilliant Red BA" (Color Index No. 621; Schultz Farbstofftabellen No. 706) was added while agitating, and the materials dyed for 15 minutes. The skins were then drawn through squeezing rolls, thoroughly rinsed in a paddle with running water, centrifuged and dried. After having placed them in damp saw dust the skins were staked and brushed on the flesh side. In this way an even yellow dyed fleshside with 40 undyed wool was obtained.

**35**  
*Example 2*  
75 skins were pretreated as described in Example 1, but left in the paddle. After addition of 1 kilogram of lauryl alcohol sulfonate the water was warmed, while agitating, to a temperature of 48° C. An aqueous solution of 1 kilogram of "Derma Brown R" (Color Index No. 518; Schultz Farbstofftabellen No. 510) was then added whereupon the further treatment was carried out 50 as indicated in Example 1.

**55**  
*Example 3*  
With a view to obtain a more penetrating dyeing, skins having been pretreated in the way disclosed in Example 1 were placed in a paddle

which contained 1000 litres of water of 48° C., 1.5-2 grams/litre of an alkyl phenyl polyglycol ether and 1 gram/litre of dyestuff and which was adjusted by means of ammonia to a pH of 9. It was dyed for about 25 minutes, but for at most 30 minutes. Afterwards the dyebath was acidified by means of formic- or acetic-acid until a pH value of 3.5 was reached, whereupon the goods were again dyed for 5-10 minutes. The further treatment was carried out according to Exam- 10

ple 1.

What we claim is:

1. In a process of dyeing a chrome tanned fur skin with reserve of the fur, the flesh side only being dyed, the step of dyeing the chrome tanned 15 fur skin with a substantive dyestuff in an aqueous solution containing a capillarily active substance selected from the group consisting of soap, oleic methyltauride, the oleic ester of hydroxyethanesulfonic acid, glycerolmonooleate ester sulfonate 20 and lauryl alcohol sulfonate at a temperature of 40 to 50° C. whereby the fur remains undyed while the flesh side is dyed.

2. In a process of dyeing a chrome tanned lamb skin with reserve of the wool thereon, the flesh 25 side only being dyed, the step of dyeing the chrome tanned lamb skin with a substantive dyestuff in an aqueous solution containing a capillarily active substance selected from the group consisting of soap, oleic methyltauride, the oleic 30 ester of hydroxyethanesulfonic acid, glycerolmonooleate ester sulfonate and lauryl alcohol sulfonate at a temperature of 40 to 50° C. whereby the wool remains undyed while the flesh side is dyed.

3. In a process of dyeing a chrome tanned sheep skin with reserve of the wool thereon, the flesh side only being dyed, the step of dyeing the chrome tanned sheep skin with a substantive dyestuff in an aqueous solution containing a capillarily active substance selected from the group consisting of soap, oleic methyltauride, the oleic ester of hydroxyethanesulfonic acid, glycerolmonooleate ester sulfonate and lauryl alcohol sulfonate at a temperature of 40 to 50° C., whereby the wool remains undyed while the flesh side is dyed.

ERNST LÜSCHER.  
ALBERT ENGELÖCH.

#### REFERENCES CITED

The following references are of record in the file of this patent:

#### UNITED STATES PATENTS

| Number    | Name      | Date          |
|-----------|-----------|---------------|
| 1,968,795 | Bertsch   | July 31, 1934 |
| 2,183,752 | Mendoza   | Dec. 19, 1939 |
| 2,228,369 | Schoeller | Jan. 14, 1941 |
| 2,254,965 | Kling     | Sept. 2, 1941 |

#### FOREIGN PATENTS

| Number  | Country       | Date          |
|---------|---------------|---------------|
| 493,781 | Great Britain | Oct. 14, 1938 |

#### OTHER REFERENCES

Chem. Trade Journal for September 1, 1933, page 155.